



US006447985B1

(12) **United States Patent**  
Thomas

(10) **Patent No.:** US 6,447,985 B1  
(45) **Date of Patent:** Sep. 10, 2002

(54) **SOLUTION TO ACCELERATE THE  
BLEACHING OF A COLOR  
PHOTOGRAPHIC PRODUCT**

(75) Inventor: **Francoise M. Thomas,**  
Chalon-sur-Saone (FR)

(73) Assignee: **Eastman Kodak Company**, Rochester,  
NY (US)

(\*) Notice: Subject to any disclaimer, the term of this  
patent is extended or adjusted under 35  
U.S.C. 154(b) by 0 days.

(21) Appl. No.: **09/705,303**

(22) Filed: **Nov. 3, 2000**

(30) **Foreign Application Priority Data**

Nov. 12, 1999 (FR) ..... 99 14473

(51) **Int. Cl.<sup>7</sup>** ..... **G03C 5/40; G03C 7/392**

(52) **U.S. Cl.** ..... **430/449**

(58) **Field of Search** ..... 430/449

(56) **References Cited**

U.S. PATENT DOCUMENTS

4,506,007 A 3/1985 Nakajima et al. ..... 430/393

4,588,471 A \* 5/1986 Griffith et al. ..... 156/652  
4,666,212 A \* 5/1987 Loveday et al. ..... 299/5  
4,913,787 A \* 4/1990 Kiso ..... 204/44.3  
4,959,278 A \* 9/1990 Shimauchi et al. ..... 428/642

FOREIGN PATENT DOCUMENTS

|    |          |        |
|----|----------|--------|
| EP | 678 783  | 4/1995 |
| EP | 679 945  | 4/1995 |
| JP | 51/95630 | 8/1978 |

\* cited by examiner

*Primary Examiner*—Hoa Van Le

(74) *Attorney, Agent, or Firm*—Andrew J. Anderson

(57) **ABSTRACT**

This invention concerns a new processing solution to accelerate the bleaching of a color photographic product. This invention further concerns a method for the processing of a photographic product that uses such a solution to accelerate the bleaching process.

The invention makes available a new solution to accelerate bleaching with improved efficacy.

**12 Claims, No Drawings**



one or more layers of silver halide emulsion and one or more additional layers. These photographic materials are described in detail in *Research Disclosure*, sections I to XVII.

The invention is described in detail in the following examples.

## EXAMPLES

### Example 1

A color cinematographic film, Vision Color Premier, marketed by Eastman Kodak, having a silver content of about 2.3 g/m<sup>2</sup> was exposed through a 21 step tablet wedge, with an increment of 0.15 log E to incident light of color temperature 2850° K. through a C1700 filter for 1/100 s. The film was then developed using the conventional Kodak ECP-2B process as described in the manual H24 (Manual for processing Eastman Color Films, module 9), wherein the bleaching step is performed using a solution of persulfate containing 30 g/l of sodium persulfate.

A first sample was processed with the bleach acceleration solution specified in the manual. This solution consisted of:

|                                |             |
|--------------------------------|-------------|
| H <sub>2</sub> O               | 800 ml      |
| Anhydrous sodium metabisulfite | 3.3 g       |
| Acetic acid (90%)              | 6.25 ml     |
| Accelerator PBA-1              | 3.3 g       |
| EDTA                           | 0.5 g       |
| H <sub>2</sub> O               | QSP 1 liter |
| Ph                             | 4           |



The processing conditions are given in Table 1.

After processing, the quantity of residual silver in the film was measured. This silver content was measured by infrared spectrophotometry at 900 nm from a calibration curve. The results are given in Table 1 below.

### Example 2

A second sample of Vision Color Premier® film was processed with the same processing solutions as in example 1, but in the treatment conditions given in Table 1 below. After processing, the quantity of residual silver was measured. The results are given in Table 1 below.

### Example 3

In this example the Vision Color Premier® photographic material was exposed and developed in the same conditions as in example 1. In this example, the bleach accelerator was modified, and consisted of:

|                                |         |
|--------------------------------|---------|
| H <sub>2</sub> O               | 800 ml  |
| Anhydrous sodium metabisulfite | 3.3 g   |
| Sodium dihydrogen phosphate    | 7 g     |
| Phosphoric acid (85%)          | 2.65 ml |
| PBA-1 accelerator              | 3.3 g   |
| EDTA                           | 0.5 g   |

-continued

|                  |             |
|------------------|-------------|
| H <sub>2</sub> O | QSP 1 liter |
| pH               | 3           |

The conditions of processing are given in Table 1.

After processing, the quantity of residual silver was measured by infrared spectrophotometry at 900 nm from a calibration curve. The results are given in Table 1 below.

### Example 4

A second sample of Vision Color Premier® film was processed with processing solutions identical to those in example 3, but in different conditions given in Table 1 below. After processing, the quantity of silver was measured. The results are given in Table 1 below.

TABLE 1

|       | Accelerator treatment time | Bleaching treatment time | Bleach temperature | Residual silver (mg/dm <sup>2</sup> ) |
|-------|----------------------------|--------------------------|--------------------|---------------------------------------|
| Ex. 1 | 20 s                       | 40 s                     | 27° C.             | 0.219                                 |
| Ex. 2 | 12 s                       | 24 s                     | 27° C.             | 3.27                                  |
| Ex. 3 | 12 s                       | 24 s                     | 27° C.             | 0.21                                  |
| Ex. 4 | 12 s                       | 24 s                     | 20° C.             | 0.83                                  |

It is known that a photographic material is considered as correctly bleached when its residual silver content is less than or equal to 0.8 mg/dm<sup>2</sup>.

These results show that when the solution of the invention is used as a bleach accelerator the residual silver content is greatly reduced even when the bleach acceleration and bleaching times are shortened (Ex. 1 and Ex. 3).

Example 2 shows that when the treatment time is reduced without modifying the pH the residual silver level is unacceptable.

Example 4 shows that the bleach accelerator solution of the invention remains efficacious at reduced processing times and lower temperatures.

These examples show that lowering the pH affords bleach accelerator solutions that make the bleaching step particularly efficacious.

The invention has been described in detail with particular reference to certain preferred embodiments thereof, but it will be understood that variations and modifications can be effected within the spirit and scope of the invention.

What is claimed is:

1. A processing solution to accelerate the bleaching of a color photographic material, that contains no bleaching agent, and that contains a bleach accelerator, wherein the pH of the solution is less than or equal to 3 and the bleach accelerator is an isothiourea of the formula:



where R<sup>1</sup> and R<sup>2</sup> are independently a hydrogen atom or an alkyl group containing from 1 to 10 carbon atoms, and n is between 1 and 4.

2. The processing solution of claim 1, wherein the quantity of bleach accelerator is at least 0.2 g/l.

3. The processing solution of claim 1, wherein the pH is in the range of from 2 to 3.

4. A method for processing a silver halide color photographic material, that includes a step of bleach acceleration of the photographic material and a step of bleaching the photographic material, wherein (i) the bleach acceleration step is separate from the bleaching step, (ii) the bleaching step is carried out with a bleaching solution containing a persulfate, and (iii) the bleach acceleration step is carried out with a solution of claim 1.

5. The method of claim 4, wherein the bleach acceleration step is carried out with a solution having a pH in the range of from 2 to 3.

6. The processing solution of claim 1, wherein the bleach accelerator has the formula



7. The processing solution of claim 6, which contains an amount of the bleach accelerator between 0.2 and 5 g/l.

8. The processing solution of claim 7, which contains 3.3 g/l of the bleach accelerator, 3.3 g/l of anhydrous sodium metabisulfite, 7 g/l of sodiumdihydrogenophosphate, 2.65 ml/l of 85% phosphoric acid, and 0.5 g/l of EDTA.

10

9. The method of claim 4, wherein the quantity of bleach accelerator in the bleach accelerator processing solution is at least 0.2 g/l.

10. The method of claim 4, wherein the bleach accelerator has the formula



15

11. The method of claim 10, wherein the bleach accelerator processing solution contains an amount of the bleach accelerator between 0.2 and 5 g/l.

12. The method of claim 11, wherein the bleach accelerator processing solution contains 3.3 g/l of the bleach accelerator, 3.3 g/l of anhydrous sodium metabisulfite, 7 g/l of sodiumdihydrogenophosphate, 2.65 ml/l of 85% phosphoric acid, and 0.5 g/l of EDTA.

20

\* \* \* \* \*